

Patented Oct. 27, 1953

2,657,135

# UNITED STATES PATENT OFFICE

2,657,135

## PHOTOGRAPHIC EMULSIONS AND SOLUTIONS CONTAINING THIOLYCOLIC ACID DERIVATIVES

Wesley G. Lowe and Marcelle E. Hamshire, Rochester, N. Y., assignors to Eastman Kodak Company, Rochester, N. Y., a corporation of New Jersey

No Drawing. Application November 5, 1949,  
Serial No. 125,846

7 Claims. (Cl. 95—7)

1

This invention relates to photography and particularly to a method of preventing image degradation of an exposed silver halide emulsion during processing.

Silver halide emulsions are frequently subject to image degradation during processing, that is, during development, fixing, washing, toning, etc., and during the moist heat to which they are subjected on drying as when prints are subjected to ferrotyping or hot-glazing. This deterioration of the image frequently manifests itself as "plumming" or "bronzing" of the image during ferrotyping. Other types of image degradation are also encountered as will become apparent hereinafter.

It is accordingly an object of our invention to provide a method for preventing image degradation of an exposed silver halide emulsion during processing. A further object is to provide a method for preventing "plumming" of exposed and developed photographic prints during ferrotyping. A further object is to provide silver halide emulsions containing agents which reduce or prevent plumping or other types of image degradation. A still further object is to provide a method for preventing or reducing various types of image deterioration during processing of an exposed silver halide layer. Other objects will appear from the following description of our invention.

These objects are accomplished by performing one or more of the steps of developing, fixing, washing and drying an exposed silver halide emulsion in the presence of a thioglycolic acid amide derivative of the following formula:



where R is any of various aryl, heterocyclic, acyl or amino groups or the acylated derivatives of these compounds. The thioglycolic acid derivatives may be present in any one or more of the processing baths or may be incorporated in the sensitive emulsion layer prior to exposure or may be incorporated in an overcoating or backing layer of the sensitive material.

The following thioglycolic acid derivatives exemplify those which may be used according to our invention.

1. 4,6 - dichloro - 5 - methyl - 2 - m - thioglycolyl - amino benzoylaminophenol
2. 2 - hydroxy - 3,5 - dichloro - 4 - methylthioglycolic anilide
3. 2 - hydroxy - 5 - chlorothioglycolic anilide
4. 2,4,6 - trichloro - 5 - thioglycolylamino phenol
5. p - thioglycolylamino -  $\omega$  - cyanoacetophenone
6. Thioglycolic anilide
7. 2 - thioglycolylamino - 4 - methyl phenol
8. 2 - thioglycolylamino - 5 - methyl phenol
9. 2 - hydroxy - 4' - thioglycolylamino diphenyl
10. 2 - thioglycolylamino phenol
11. 2 - (p - thioglycolylaminophenylacetamino) - 4,6 - dichloro - 5 - methyl phenol
12. 4 - nitrothioglycolyl anilide
13. 2,4 - dichlorothioglycolyl anilide
14. Thioglycolyl - 4 - iodo anilide
15. Thioglycolic - 4 - sulfamido anilide
16. Thioglycolic - 4 - cyano anilide
17. Thioglycolic - 2,5 - dichloro anilide
18. 5 - thioglycolylamino - 1 - naphthol
19. 2 - (thioglycolylamino) benzothiazole
20. 5 - thioglycolylaminotetrazole
21. 2 - thioglycolylaminopyrimidine
22. 5 - thioglycolylamino - 1,2,4 - triazole
23. Thioglycolylurea
24. Thioglycolic -  $\omega$  - aminocapramide
25. Thioglycolic hydrazide
26. Thioglycolic - 2,6 - dihydroxy anilide

When incorporated in silver halide emulsions, these compounds are preferably used in a gelatinous silver chloride emulsion or a silver chloride emulsion containing small amounts of bromide or iodide. Silver halide emulsions in which the carrier is polyvinyl alcohol or hydrolyzed cellulose acetate may also be used. When the thioglycolic derivatives are incorporated in the emulsion, they should be used in amounts of from about 2.5 to 25 grams per unit of silver halide formed from 1000 grams of silver nitrate. The same concentration of the agents should be present in the emulsion when the agents are added by bathing the emulsion in a solution containing them. When the emulsion layer is bathed in a solution of the compound, the solution may contain up to about 5% of the compound.

Not all of the compounds used according to our invention are equally effective for preventing or reducing all types of image degradation, although the listed compounds have been found to have some value in most cases. For preventing plumping, that is, loss of reflection density or tone change on hot ferrotyping of photographic prints, all of the specific compounds listed above are effective. The acylated derivatives of these compounds are less effective in general, although the following acylated compounds have been found to be very satisfactory in anti-plumping action.

- 4,6 - dichloro - 5 - methyl - 2 - m - acetyl thioglycolylaminobenzoylaminophenol,
- 5 - acetylthioglycolylamino - 1 - naphthol,
- 2 - (acetyl thioglycolylamino) benzothiazole.

A further use of our compounds is in image protecting action, that is, stabilization of the developed image against chemical attack by such reagents as dilute cyanide or sodium thiosulfate or ammonium thiosulfate solutions such as used in fixing baths. In general, all of the compounds listed above are suitable for this purpose.

A further use of our compounds is for contrast increasing, desensitizing and stabilizing action, especially where the compounds are incorporated in the sensitive emulsion layer. Compounds 7, 8, 18, 23, 24 and 26 are especially suitable for this purpose.

Compound 25 is very effective for desensitizing and stabilizing action without raising contrast when the compound is incorporated in the emulsion.

Compound 25 is also effective in preventing "hypo drag" that is, erratic tone changes in the print when placed into hypo without adequate 20 washing after development. A still further use of our compounds is in cold toning, that is, in producing blue-black tones upon processing the emulsion layer. Compounds 16, 19, 20, 21, 22 and 23 are especially suitable for this purpose as 25 are the following acetylated compounds:

2-(acetylthioglycolylamido)benzothiazole

5-acetylthioglycolylaminotetrazole

2-acetylthioglycolylaminopyrimidine

Acetothioglycolyl-4-cyanoamide

We are aware that thioglycolic anilides have been used in photographic emulsions as described, for example, in Weissberger, Kibler and Young U. S. Patent 2,448,939. In that case, however, the compounds were used for color-forming purposes and were added to the emulsion in much larger amounts than are used according to the present invention. No image degradation prevention was sought or obtained in the Weissberger, Kibler and Young process with the large amount of thioglycolic compound used. Since the silver is usually removed in a color process, silver is not present after processing and during ferrotyping so that no image protecting action would be required or obtained.

We claim:

1. The method of preventing image degradation of an exposed silver halide emulsion during processing, which comprises developing, fixing, washing and drying said emulsion, and performing at least one of the steps of developing, fixing, washing and drying said emulsion in the presence in said emulsion of from 2.5 grams to 25 grams per unit of silver halide formed from 1000 grams of silver nitrate, of a compound selected from those compounds having the formula

R—NHCOCH<sub>2</sub>SH

where R is selected from the class consisting of aryl, heterocyclic and acyl groups and the acetylated derivatives of said compounds.

2. The method of preventing image degradation of an exposed silver halide emulsion during processing, which comprises developing, fixing, washing and drying said emulsion, and incorporating in at least one of the developing, fixing and washing baths used to process said emulsion, an appreciable amount but less than 5%, of a compound having the general formula

R—NHCOCH<sub>2</sub>SH

where R is an aryl group, and processing said exposed emulsion in said bath.

3. The method of preventing image degradation of an exposed silver halide emulsion during

processing, which comprises developing, fixing, washing and drying said emulsion, and incorporating in at least one of the developing, fixing and washing baths used to process said emulsion, an appreciable amount but less than 5%, of a compound having the general formula

R—NHCOCH<sub>2</sub>SH

where R is a heterocyclic group, and processing said exposed emulsion in said bath.

4. The method of preventing image degradation of an exposed silver halide emulsion during processing, which comprises developing, fixing, washing and drying said emulsion, and incorporating in at least one of the developing, fixing and washing baths used to process said emulsion, an appreciable amount but less than 5%, of a compound having the general formula

R—NHCOCH<sub>2</sub>SH

where R is an acyl radical, and processing said exposed emulsion in said bath.

5. A photographic silver halide emulsion containing from 2.5 to 25 grams per unit of silver halide formed from 1000 grams of silver nitrate, of a compound selected from those compounds having the formula

R—NHCOCH<sub>2</sub>SH

where R is selected from the class consisting of aryl, heterocyclic and acyl groups, and the acetylated derivatives of said compounds.

6. A photographic silver halide emulsion containing from 2.5 to 25 grams per unit of silver halide formed from 1000 grams of silver nitrate, of a thioglycolylamino heterocyclic compound.

7. A photographic silver halide emulsion containing from 2.5 to 25 grams per unit of silver halide formed from 1000 grams of silver nitrate, of a compound selected from the group consisting of 4,6 - dichloro - 5 - methyl - 2 - m - thioglycolylaminobenzoylaminophenol, 2 - hydroxy-3,5 - dichloro - 4 - methylthioglycolic anilide, 2-hydroxy - 5 - chlorothioglycolic anilide, 2,4,6-trichloro - 5 - thioglycolylamino phenol, p - thioglycolylamino -  $\omega$  cyanoacetophenone, thioglycolic anilide, 2 - thioglycolylamino - 4 - methyl phenol, 2 - thioglycolylamino - 5 - methyl phenol, 2 - hydroxy - 4' - thioglycolylamino diphenyl, 2 - thioglycolylamino phenol, 2 - (p - thioglycolylaminophenyl-acetamino) - 4,6 - dichloro-5 - methyl phenol, 4 - nitrothioglycolyl anilide, 2,4 - dichlorothioglycolyl anilide, thioglycolyl-4-iodo anilide, thioglycolic - 4 - sulfamido anilide, thioglycolic - 4 - cyano anilide, thioglycolic - 2,5-dichloroanilide, 5-thioglycolylamino-1-naphthol, 2 - (thioglycolylamino)benzothiazole, 5 - thioglycolylaminotetrazole, 2 - thioglycolylaminopyrimidine, 5 - thioglycolylamino - 1,2,4 - triazole, thioglycolylurea, thioglycolic- $\omega$ -aminocapramide, and thioglycolic-2,6-dihydroxy anilide.

WESLEY G. LOWE.

MARCELLE E. HAMSHIRE.

References Cited in the file of this patent

UNITED STATES PATENTS

| Number    | Name        | Date          |
|-----------|-------------|---------------|
| 1,673,522 | Matthies    | June 12, 1928 |
| 1,758,576 | Matthies    | May 13, 1930  |
| 2,448,939 | Weissberger | Sept. 7, 1948 |
| 2,453,346 | Russell     | Nov. 9, 1948  |

FOREIGN PATENTS

| Number  | Country       | Date          |
|---------|---------------|---------------|
| 631,184 | Great Britain | Oct. 28, 1949 |